# EUROPEAN PATENT SPECIFICATION

(11) **EP 0 571 470 B1**
(45) Date of publication and mention of the grant of the patent: **02.08.1995**
(21) Application number: 92904830.4
(22) Date of filing: 16.12.1991
(51) Int. Cl.: C11D 1/835, C11D 17/04, D06M 10/08

(54) **LAUNDRY RINSES AND DRYER SHEETS**
WÄSCHESPÜLMITTEL UND BLÄTTER FÜR GEWEBETRÖCKNER
PRODUIT DE RINCAGE ET FEUILLES DE SECHAGE DE LESSIVE

(30) Priority: 08.02.1991 US 652602; 08.02.1991 US 652615; 08.02.1991 US 652619
(43) Date of publication of application: 01.12.1993
(73) Proprietor: ALBEMARLE CORPORATION, Richmond, Virginia 23219 (US)
(72) Inventor: CRUTCHER, Terry, Baton Rouge, LA 70810 (US); SMITH, Kim, R., Baton Rouge, LA 70810 (US); BORLAND, James, E., Baton Rouge, LA 70815 (US); SAUER, Joe, D., Baton Rouge, LA 70816 (US); PERINE, Jeffrey, W., Baton Rouge, LA 70810 (US)
(74) Representative: Sandmair, Kurt, Dr. Dr.
(86) International application number: US9109453
(87) International publication number: WO9213934

(56) References cited:
- EP-A- 0 052 972
- DE-A- 2 000 231
- DE-A- 2 426 581
- GB-A- 2 240 791
- US-A- 3 843 395
- US-A- 4 264 457
- US-A- 5 080 810

## Description

### Field of Invention

This invention relates to laundry rinses and dryer sheets containing N,N-dihydrogenatedtallow-N,N-dimethylammonium chloride and an amine oxide.

### Background

When fabrics are laundered, it is frequently desirable to treat them with fabric softeners, not only to soften them, but to give them greater bulk, make them easier to iron, decrease fabric drying time, and reduce static charge. A fabric softener that is commonly used is N,N-dihydrogenatedtallow-N,N-dimethylammonium chloride (DTMAC), which is both inexpensive and effective as a softener but, on the other hand, has certain deficiencies, such as its yellowing and reducing the washability of the softened fabrics, having inefficient antistatic activity on polyesters, and decreasing the rewettability of the treated fabrics.

Amine oxides, such as N-alkyl-N,N-dimethylamine oxides, are also effective fabric softeners; and they sometimes have advantages over DTMAC in this regard. However, when used together with DTMAC, they have either failed to improve the results obtained with DTMAC alone or have provided results intermediate to those obtained with either component of the fabric softener alone.

As one examplary approach US-A-3 843 395 addresses the improvement of fabric softening compositions with respect to staining of laundry. To fulfil this object the softening composition is impregnated into an absorbent material. However, the softening compounds may be chosen from a broad range of compounds including 9 general formulae and thus 9 different classes of compounds which may be used alone or in combinations thereof.

### Summary of Invention

It has now been found that the use of an N-octadecyl-N,N-dimethylamine oxide together with N,N-dihydrogenatedtallow-N,N-dimethylammmonium chloride can provide an improved fabric softener product when the fabric softener product is (1) a laundry rinse which comprises as the sole fabric softener an aqueous solution of a mixture of 25-80% of the by weight of the quaternary ammonium chloride and 75-20% by weight of the amine oxide or (2) a laundry dryer sheet which comprises a flexible absorbent substrate impregnated with a fabric softener that is a mixture of 10-80% by weight of the quaternary ammonium chloride and 90-20% by weight of the amine oxide.

### Detailed Description

As already mentioned, the quaternary ammonium chloride component of the fabric softener mixture is the known N,N-dihydrogenatedtallow-N,N-dimethylammonium chloride (DTMAC). The DTMAC used in preparing the mixture is generally the material that is most commonly available, i.e., a 75% paste in an alcohol.

The amine oxide component of the mixture is N-octadecyl-N,N-dimethylamine oxide.

Although the amine oxide used in preparing any of the products of the invention may be a conventional aqueous solution or a solid amine oxide, such as the amine oxide dihydrates described in European Patent Application 0401503 and British Patent Application 2,240,791, it is apt to be preferred to employ an amine oxide in solution form when the mixture is to be utilized as an aqueous solution and otherwise to employ a solid amine oxide.

Except for the fabric softener mixture used, a laundry rinse of the invention is a conventional rinse which has water as its major ingredient (generally comprising 70-90% by weight of water) and may contain any of the other ingredients typically used in laundry rinses, e.g., minor amounts of materials such as dyes and perfumes and sometimes an alcohol, such as ethanol, to prevent phase separation, as well as the novel fabric softener mixture. Moreover, the rinse may be prepared as such rinses are normally prepared except for the use of the novel mixture as the fabric softener; and conventional techniques are also suitable for rinsing laundry therewith.

All of the laundry rinses of the invention, regardless of the particular proportionation of DTMAC and N-octadecyl-N,N-dimethylamine oxide within the specified ranges, have the advantage of providing laundered fabrics, such as cotton, with better rewettability than laundry rinses containing only one component of the fabric softener mixture; but optimum rewettability is obtained when the fabric softener is a mixture of 75% by weight of the quaternary ammonium chloride and 25% by weight of the amine oxide. This advantage of the mixtures is unexpected, since such synergism is not obtained when other amine oxides, such as N-octyl-N,N-dimethylamine oxide, are used instead of the N-octadecyl-N,N-dimethylamine oxide.

A laundry dryer sheet of the invention may be prepared by the conventional technique of soaking an absorbent flexible substrate with an aqueous mixture of the fabric softener mixture, pressing the resultant soaked sheet to remove any excess surfactant, and then drying it. However, it is preferably prepared by coating an absorbent flexible substrate with a molten mixture of the fabric softener components and then solidifying the mixture.

In preparing a laundry dryer sheet from a molten fabric softener mixture, it is convenient to conduct the process by soaking the absorbent flexible substrate in a molten mixture of the fabric softener components, thus coating and inherently impregnating it with the surfactants; passing the soaked sheet between two rollers, as in a roller press, to remove any excess surfactant; and allowing the remaining surfactant to solidify.

The absorbent flexible substrate used in preparing the dryer sheets may be any of the substrates typically employed in making such sheets, since the only requirement for the substrate is that it be an absorbent material in sheet form. For example, it may be a sponge, paper, or woven or non-woven cloth, especially a non-woven cloth made from fibers or filaments of a material such as wool, silk, jute, hemp, cotton, linen, sisal, ramie, rayon, cellulose esters, vinyl polymers, polyamides, and polyesters. A particularly desirable substrate is a sheet of non-woven polyethylene terephthalate cloth.

All of the laundry dryer sheets of the invention in which the fabric softener is a mixture of 50-80% by weight of DTMAC and 50-20% by weight of N-octadecyl-N,N-dimethylamine oxide have the advantage of being able to impart greater softness to laundered fabrics, such as cotton, than can be achieved when either component of the mixture is used alone as the fabric softener. However, optimum reults are achieved when the fabric softener is a mixture of 75% by weight of DTMAC and 25% by weight of the amine oxide.

The laundry dryer sheets in which the fabric softener is a mixture of 10-60% by weight of DTMAC and 90-40% by weight of any of the aforementioned N-octadecyl-N,N-dimethylamine oxide have the advantage of leading to the reduction of static charge buildup on laundered polyester fabrics or laundry batches comprising at least some polyester fabric when they are used in the drying step. In this case, optimum results are obtained when the fabric softener is a mixture of 50% by weight of DTMAC and 50% by weight of the amine oxide.

The following examples are given to illustrate the invention and are not intended as a limitation thereof. Unless otherwise specified, quantities mentioned in the examples are quantities by weight.

### EXAMPLE I

Five medium-grade cotton terrycloth towels were subjected to four wash/rinse/dryer cycles in which the rinses were aqueous solutions of N-octadecyl-N,N-dimethylamine oxide (AO-18) and/or N,N-dihydrogenatedtallow-N,N-dimethylammonium chloride (DTMAC). The treated towels were then tested for rewettability in accordance with CSMA test protocol Method D-13D by cutting the towels into strips measuring 5 x 6 inches (12.7 x 15.2 cm), marking each of the strips one centimeter from the narrow edge and lowering it into a 0.01% Rhodamine B dye bath for six minutes, and recording the distance of dye movement at the end of that time in centimeters. The amounts of AO-18 and DTMAC used in the fabric softener and the results of the rewettability tests are shown in the Table following the examples.

### EXAMPLE II

Fifty cotton hand-towels were washed on medium loading for 30 minutes in the presence of 37.5g of an anionic laundry detergent and divided into five groups of ten towels, each group then being loaded into an automatic dryer and dried for 60 minutes on "normal" at about 65° C in the presence of a polyester dryer sheet having a 1g loading of softener comprising AO-18 and/or DTMAC. The softness of the dried towels was then evaluated by a panel of evaluators who ranked them from 5 (softest) to 1 (least soft). The amounts of AO-18 and DTMAC used in the fabric softener and the results of the softness test are shown in the Table following the examples.

### EXAMPLE III

A laundry batch composed of 23% polyester fabric, 46% cotton/polyester fabric, and 31% cotton fabric was washed on medium loading for 30 minutes in the presence of an anionic laundry detergent and then separated into five identical sub-batches. Each sub-batch was loaded into an automatic dryer, a polyester dryer sheet having a 1g loading of AO-18 and/or DTMAC fabric softener was placed into each of the automatic dryers on top of the sub-batch, and the sub-batch was then dried for 60 minutes on "normal" at about 65° C. The antistatic activity of the fabric softener in each dryer sheet was then determined in accordance with CSMA test protocol Method D-13F by removing the separate pieces of laundered fabric from the dryer, dropping them into a Faraday cage, and recording the initial voltage -- the test being performed on a day when the relative humidity was 50% at 22° C. The amounts of AO-18 and DTMAC used in the fabric softener and the results of the softness test are shown in the Table following the examples.

**TABLE**

| % AO | % DTMAC | Dye Movement (cm) | Softness | Static Charge (kV) | |
|---|---|---|---|---|---|
| | | | | Overall | Polyester |
| 100 | 0 | 2.8 | 2.7 | 3.8 | 1.3 |
| 75 | 25 | 4.0 | 2.5 | 1.2 | 1.3 |
| 50 | 50 | 4.4 | 3.3 | 1.5 | 0.1 |
| 25 | 75 | 4.8 | 3.6 | 3.1 | 1.7 |
| 0 | 100 | 1.6 | 3.0 | 2.8 | 1.7 |

## Claims

1. A fabric softener containing N,N-dihydrogenatedtallow-N,N-dimethylammonium chloride and N-octadecyl-N,N-dimethylamine oxide, characterized in that it is (1) a laundry rinse which comprises as the sole fabric softener an aqueous solution of a mixture of 25-80% by weight of the substituted ammonium chloride and 75-20% by weight of the amine oxide or (2) a laundry dryer sheet which comprises a flexible absorbent substrate impregnated with a fabric softener that is a mixture of 10-80% by weight of the substituted ammonium chloride and 90-20% by weight of the amine oxide.

2. The fabric softener product of claim 1 which is a laundry rinse.

3. The fabric softener product of claim 1 which is a laundry dryer sheet comprising a flexible absorbent substrate impregnated with a mixture of 50-80% by weight of the substituted ammonium chloride and 50-20% by weight of the amine oxide as a fabric softener.

4. The fabric softener product of claim 2 or 3 wherein the fabric softener is a mixture of 75% by weight of the substituted ammonium chloride and 25% by weight of the amine oxide.

5. The fabric softener product of claim 1 which is a laundry dryer sheet comprising a flexible absorbent substrate impregnated with a mixture of 10-60% by weight of the substituted ammonium chloride and 90-40% by weight of the amine oxide as a fabric softener.

6. The fabric softener product of claim 5 wherein the fabric softener is a mixture of 50% by weight of the substituted ammonium chloride and 50% by weight of the amine oxide.

7. A process for providing softened laundered fabrics having improved rewettability tested in accordance with CSMA test protocol Method D-13D, which comprises rinsing the laundry fabrics with a laundry rinse of claim 1.

8. A process for improving the softness of a laundered fabric which comprises drying the laundered fabric in an automatic dryer containing a laundry dryer sheet of claim 3 or 4.

9. A process for reducing static charge buildup on a laundry batch comprising at least some polyester fabric which comprises drying the laundry batch in an automatic dryer containing a laundry dryer sheet of claim 5 or 6.

## Patentansprüche

1. Weichmacher für Stoffe (Weichspüler), der N,N-dihydriertes Talg-N,N-dimethylaminochlorid und N-Octadecyl-N,N-dimethylaminoxid enthält, dadurch gekennzeichnet, daß es sich (1) um einen Wäschespüler, der als einzigen Stoffweichmacher eine wäßrige Lösung einer Mischung aus 25 bis 80 Gew. -% des substituierten Ammoniumchlorids und 75 bis 20 Gew. -% des Aminoxids enthält, (2) um ein Flauschtuch (Wäschetrocknerblatt) handelt, das ein biegsames absorptionsfähiges, mit einem Stoffweichmacher imprägniertes Substrat enthält, der eine Mischung aus 10 bis 80 Gew. -% des substituierten Ammoniumchlorids und 90 bis 20 Gew. -% des Aminoxids ist.

2. Stoffweichmacherprodukt nach Anspruch 1, bei dem es sich um einen Wäschespüler handelt.

3. Stoffweichmacherprodukt nach Anspruch 1, bei dem es sich um ein Flauschtuch (Wäschetrocknerblatt) handelt, das ein biegsames absorptionsfähiges, mit einer Mischung aus 50 bis 80 Gew.-% des substituierten Ammoniumchlorids und 50 bis 20 Gew. -% des Aminoxids als Stoffweichmacher imprägniertes Substrat enthält.

4. Stoffweichmacherprodukt nach Anspruch 2 oder 3, bei dem der Stoffweichmacher eine Mischung aus 75 Gew. -% des substituierten Ammoniumchlorids und 25 Gew. -% des Aminoxids ist.

5. Stoffweichmacherprodukt nach Anspruch 1, bei dem es sich um ein Flauschtuch (Wäschetrocknerblatt) aus einem biegsamen, absorptionsfähigen, mit einer Mischung aus 10 bis 60 Gew. -% des substituierten Ammoniumchlorids und 90 bis 40 Gew. -% des Aminoxids als Stoffweichmacher imprägnierten Substrat handelt.

6. Stoffweichmacherprodukt nach Anspruch 5, bei dem der Stoffweichmacher eine Mischung aus 50 Gew. -% des substituierten Ammoniumchlorids und 50 Gew. -% des Aminoxids ist.

7. Verfahren, um weichgespülte gewaschene Stoffe mit verbesserter Wiederbenetzbarkeit zur Verfügung zu stellen, welche gemäß dem CSMA Test-Protokoll, Verfahren D-13D getestet wurde, bei dem die gewaschenen Stoffe mit einem Wäschespüler nach Anspruch 1 gespült wurden.

8. Verfahren zur Verbesserung der Weichheit eines gewaschenen Stoffs, bei dem der gewaschene Stoff in einem ein Flauschtuch nach Anspruch 3 oder 4 enthaltenden Trockenautomat getrocknet wird.

9. Verfahren zur Verringerung der statischen Aufladung in einer Wäscheladung mit mindestens einem Anteil an Polyesterfasern, bei dem die Wäscheladung in einem ein Flauschtuch gemäß Anspruch 5 oder 6 enthaltenden Trockenautomat getrocknet wird.

## Revendications

1. Produit assouplisseur d'étoffes, contenant du chlorure de N,N-suif dihydrogéné-N,N-diméthylammonium et de l'oxyde de N-octadécyl-N,N-diméthylamine, caractérisé en ce qu'il consiste en (1) un produit de rinçage pour blanchisserie, qui comprend, comme seul produit assouplisseur d'étoffes, une solution aqueuse d'un mélange de 25 à 80 % en poids du chlorure d'ammonium substitué et de 75 à 20 % en poids de l'oxyde d'amine, ou (2) une feuille de séchage pour blanchisserie, qui comprend un substrat absorbant flexible imprégné avec un produit assouplisseur d'étoffes qui consiste en un mélange de 10 à 80 % en poids de chlorure d'ammonium substitué et de 90 à 20 % en poids de l'oxyde d'amine.

2. Produit assouplisseur d'étoffes suivant la revendication 1, qui est un produit de rinçage pour blanchisserie.

3. Produit assouplisseur d'étoffes suivant la revendication 1, qui est une feuille de séchage pour blanchisserie comprenant un substrat absorbant flexible imprégné avec un mélange de 50 à 80 % en poids du chlorure d'ammonium substitué et de 50 à 20 % en poids de l'oxyde d'amine, servant de produit assouplisseur d'étoffes.

4. Produit assouplisseur d'étoffes suivant la revendication 2 ou 3, l'assouplisseur d'étoffes consistant en un mélange de 75 % en poids du chlorure d'ammonium substitué et de 25 % en poids de l'oxyde d'amine.

5. Produit assouplisseur d'étoffes suivant la revendication 1, qui est une feuille de séchage pour blanchisserie comprenant un substrat absorbant flexible imprégné avec un mélange de 10 à 60 % en poids du chlorure d'ammonium substitué et de 90 à 40 % en poids de l'oxyde d'amine, servant d'assouplisseur d'étoffes.

6. Produit assouplisseur d'étoffes suivant la revendication 5, l'assouplisseur d'étoffes consistant en un mélange de 50 % en poids du chlorure d'ammonium substitué et de 50 % en poids de l'oxyde d'amine.

7. Procédé pour obtenir des étoffes blanchies assouplies présentant une remouillabilité améliorée par un essai suivant la méthode D-13D du protocole d'essai CSMA, qui comprend le rinçage des étoffes de blanchisserie avec un produit de rinçage pour blanchisserie suivant la revendication 1.

8. Procédé pour améliorer la souplesse d'une étoffe blanchie, qui comprend le séchage de l'étoffe blanchie dans un appareil automatique de séchage contenant une feuille de séchage pour blanchisserie suivant la revendication 3 ou 4.

9. Procédé pour réduire l'accumulation de charges statiques sur un lot d'étoffes de blanchisserie comprenant au moins un certain type d'étoffe à base de polyester, qui comprend le séchage du lot d'étoffes de blanchisserie dans un appareil automatique de séchage contenant une feuille de séchage pour blanchisserie suivant la revendication 5 ou 6.
